

**[54] POLYPHENYL THIOETHER LUBRICATING COMPOSITIONS****[75] Inventor:** Frank S. Clark, St. Louis, Mo.**[73] Assignee:** Monsanto Company, St. Louis, Mo.**[22] Filed:** Dec. 28, 1970**[21] Appl. No.:** 102,152**[52] U.S. Cl.** ..... 252/46.7, 252/46.6, 252/49.8,  
260/502.4 R**[51] Int. Cl.** ..... C10m 1/48**[58] Field of Search** ..... 252/45, 48.4, 46.6, 46.7**[56] References Cited****UNITED STATES PATENTS**

|           |        |                |                |
|-----------|--------|----------------|----------------|
| 2,174,019 | 9/1939 | Sullivan       | ..... 252/49.8 |
| 2,274,291 | 2/1942 | Clayton et al. | ..... 252/49.8 |
| 2,730,499 | 1/1956 | Pokorny        | ..... 252/49.8 |

|           |         |                 |                  |
|-----------|---------|-----------------|------------------|
| 2,957,931 | 10/1960 | Hamilton et al. | ..... 252/49.8 X |
| 3,426,075 | 2/1969  | Campbell        | ..... 252/45     |

**FOREIGN PATENTS OR APPLICATIONS**

851,651 10/1960 Great Britain

*Primary Examiner*—Daniel E. Wyman*Assistant Examiner*—W. Cannon*Attorney*—Neal E. Willis, J. E. Maurer and William T. Black**[57] ABSTRACT**

Lubricating compositions comprising polyphenyl thioethers, polyphenyl ethers-thioethers or mixtures thereof and containing small amounts of an organic phosphinic acid have improved lubricating properties. These compositions are useful as lubricants over wide temperature ranges.

**5 Claims, No Drawings**

## POLYPHENYL THIOETHER LUBRICATING COMPOSITIONS

This invention relates to improved lubricating compositions comprising polyphenyl thioethers, mixed polyphenyl esters-thioethers and mixtures thereof, containing from three to eight aromatic groups and a small amount of an organic phosphinic acid as a lubricating additive.

Polyphenyl thioethers and polyphenyl ether-thioether combinations have found wide application as functional fluids due to their excellent thermal stability and lubricity. For example they have been found to be valuable as hydraulic fluids and as lubricants in motor operation, particularly in jet engines.

Development of synthetic base stocks such as the polyphenyl thioether has provided lubricant fluids which are useful at elevated temperature such as 400° to 500° F. It is known that one of the aspects in which the polyphenyl thioether base stocks are considered deficient is in their lubricating characteristics, especially for steel on steel, steel on silvered bronze, or steel on cast iron. These lubricating characteristics include the load-carrying abilities and wear properties. Thus there is a demand for additives for polyphenyl thioethers which will improve the lubricity of the polyphenyl thioethers for steel on the above metallurgy.

An object of the present invention is to provide for improved lubricating compositions employing polyphenyl thioethers, polyphenyl ether-thioethers, or mixtures thereof as base stocks.

These and other objects will become evident upon consideration of the following specification and examples.

It has now been found that compositions consisting essentially of a major amount of a polyphenyl thioether base fluid having the formula



wherein R is a phenyl group, an alkyl-substituted phenyl group wherein the alkyl group contains one to four carbon atoms, an alkoxy-substituted phenyl group wherein the alkoxy group contains one to four carbon atoms or a halogenated phenyl group wherein the halogen is bromine, fluorine or chlorine, R' is a phenylene group, an alkyl or alkoxy-substituted phenylene group where the alkyl group contains one to four carbon atoms or a halogenated phenylene group wherein the halogen is fluorine, bromine or chlorine, and Y is selected from oxygen and sulfur but at least one of the Y's is sulfur and n is an integer having a value of from one to six and an additive amount of an aryl phosphinic acid have unusual ability to lubricate steel on cast iron, silver plated bronze, or steel.

The amount of the organic phosphinic acid employed in the compositions of this invention is from about 0.05 to about 2.0 percent by weight of the total composition. It is preferred to employ the aryl phosphinic acid in the compositions of this invention in amounts of from about 0.075 to about 0.2 percent by weight of the total composition.

The improvement in lubricity characteristics achieved by the addition of the aryl phosphinic acid to the polyphenyl thioether base fluid is unusual and surprising. Wear on a silver plated bronze bearing surface

is decreased at test temperatures of 645° F. whereas when the base fluid is tested without the additive the lubricity of the base fluid is not sufficient and the bearing surface fails after a short time.

5 The organic phosphinic acids which are employed in the compositions of this invention are those of the formula

10 (II)



15 wherein R'' is an aryl group containing from six to 16 carbon atoms, halogen substituted aryl groups or an alkyl group containing one to 12 carbon atoms or halogen substituted alkyl groups. Illustrative of the groups represented by R'' are, for example, phenyl,

20 tolyl, xylol, naphthyl,  $\alpha$ -methyl naphthyl and diphenyl, and aryl groups substituted with halogen or with alkyl groups containing from one to 10 carbon atoms. Such alkyl substituted aryl groups are tolyl, xylol,  $\alpha$ -methyl naphthyl, nonylphenyl, ethylphenyl, butylphenyl, t-butylphenyl and the like. Such halogen substituted aryl

25 groups are o-, m- and p-chlorophenyl, o-, m- and p-bromophenyl, the fluorophenyl groups and the like. Illustrative of the alkyl groups represented by R'' are, for example, methyl, ethyl, propyl, isopropyl, butyl, t-butyl, hexyl, isoctyl, decyl, dodecyl and the like. Such organic phosphinic acids are, for example, phenyl phosphinic acid, nonylphenyl phosphinic acid, tolyl phosphinic acid, xylol phosphinic acid, naphthyl phosphinic acid, diphenyl phosphinic acid and the like. It is

30 particularly preferred to employ in the compositions of this invention organic phosphinic acids wherein R'' is an aryl group within the above-defined definition.

35 The polyphenyl thioethers employed in the composition of this invention have from three to eight benzene rings and from one to seven sulfur atom with the sulfur atoms joining the benzene rings in chains as ether linkages.

40 By the term "polyphenyl thioether" as used herein is meant a compound or physical mixture of compounds represented by Formula I. The term includes compounds wherein all of the Y's in Formula I are sulfur. The term also includes those compounds which contain both oxygen and sulfur linkages between the benzene rings.

45 The compositions of this invention contain a major amount of the polyphenyl thioether base stock, i.e., at least 50 percent by weight of the total composition

50 comprises a polyphenyl thioether. It is preferred that at least 60 percent by weight of the composition be a polyphenyl thioether base stock and even more preferred that at least 85 percent by weight of the total composition comprise a polyphenyl thioether.

55 The compositions of this invention can also contain from 0.01 to 10 percent by weight of the total composition of a dialkyl hydrogen phosphite extreme pressure additive. The dialkyl hydrogen phosphites useful are those wherein the alkyl groups contain from one to 12 carbon atoms. These alkyl groups are for example, methyl, ethyl, propyl, isopropyl, butyl, secbutyl, t-butyl, hexyl, decyl, isodecyl, dodecyl and the like.

60 The compositions of this invention can also contain from 0.01 to 10 percent by weight of the total composition of a dialkyl hydrogen phosphite extreme pressure additive. The dialkyl hydrogen phosphites useful are those wherein the alkyl groups contain from one to 12 carbon atoms. These alkyl groups are for example, methyl, ethyl, propyl, isopropyl, butyl, secbutyl, t-butyl, hexyl, decyl, isodecyl, dodecyl and the like.

Illustrative of the alkyl-substituents present in the phenyl and phenylene groups of the polyphenyl thioethers are for example, methyl, ethyl, propyl, butyl and the like. Illustrative of the alkoxy-substituents are, for example, methoxy, ethoxy, propoxy, butoxy, and their isomers.

Illustrative of the polyphenyl thioethers which can be employed as base stocks for the compositions of this invention are the bis(phenylmercapto)benzenes. For example

bis(m-phenylmercapto)benzene  
 bis(o-phenylmercapto)benzene  
 bis(p-phenylmercapto)benzene  
 bis(m-phenylmercaptophenyl)sulfide  
 bis(o-phenylmercaptophenyl)sulfide  
 bis(p-phenylmercaptophenyl)sulfide  
 (m-phenylmercaptophenyl) (o-phenylmercapto-  
 phenyl)sulfide  
 p-phenylmercapto-m'-phenylmercapto diphenyl sul-  
 fide  
 o-bis(o-phenylmercaptophenylmercapto)benzene  
 p-bis(p-phenylmercaptophenylmercapto)benzene  
 p-bis(o-phenylmercaptophenylmercapto)benzene  
 p-bis(m-phenylmercaptophenylmercapto)benzene  
 m-bis(p-phenylmercaptophenylmercapto)benzene  
 o-bis(p-phenylmercaptophenylmercapto)benzene  
 and the like and mixtures thereof.

Illustrative of the mixed polyphenyl ether-thioether compounds which can be employed as base stocks in the compositions of this invention are for example,

o-phenylmercapto-m-phenoxy benzene  
 p-phenylmercapto-o-phenoxy benzene  
 m-phenoxy-p-phenylmercapto benzene  
 o-phenylmercapto-p'-phenoxydiphenyl sulfide  
 o-phenylmercapto-m'-phenoxydiphenyl sulfide  
 o-phenoxy-m'-phenylmercaptodiphenyl sulfide  
 m-phenoxy-p'-phenylmercaptodiphenyl sulfide  
 o-phenoxy-p'-phenylmercaptodiphenyl sulfide  
 p-phenoxy-p'-phenylmercaptodiphenyl sulfide  
 o-phenoxy-o'-phenylmercaptodiphenyl sulfide  
 o,o'-bis(phenylmercapto)diphenyl ether  
 o-phenylmercapto-m-phenylmercaptodiphenyl ether  
 o-phenylmercapto-p-phenylmercaptodiphenyl ether  
 m-(m-phenylmercaptophenylmercapto) (m-phenoxy-  
 phenyl-mercapto)benzene  
 [m-(m-phenylmercaptophenylmercapto)phenyl]  
 [m-(m-phenoxyphenylmercapto)phenyl] sulfide  
 3-(m-phenylmercaptophenylmercapto)-3'-(m-phenyl-  
 mercaptophenoxy)diphenyl sulfide  
 3,3'-bis(m-phenylmercaptophenylmercapto)diphe-  
 nyl ether  
 3-(m-phenylmercaptophenylmercapto)-3'-(m-  
 phenoxyphenoxy)diphenyl sulfide  
 4-(m-phenylmercaptophenylmercapto)-4'-(m-phenyl-  
 mercaptophenoxy)diphenyl ether  
 3-(m-phenylmercaptophenylmercapto)-3'-(m-  
 phenoxyphenylmercapto)diphenyl ether  
 4,4'-bis(m-phenylmercaptophenoxy)diphenyl sul-  
 fide  
 4,4'-bis(m-phenoxyphenylmercapto)diphenyl sul-  
 fide  
 3-(m-phenoxyphenylmercapto)-3'-(m-phenylmer-  
 captophenoxy)diphenyl sulfide  
 3,3'-bis(m-phenylmercaptophenoxy)diphenyl ether  
 4-(m-phenylmercaptophenylmercapto)-4'-(m-  
 phenoxyphenoxy)diphenyl ether

3-(p-phenylmercaptophenoxy)-3'-(p-phenoxy-  
 phenoxy)diphenyl sulfide  
 3-(m-phenylmercaptophenoxy)-3'-(m-phenoxy-  
 phenylmercapto)diphenyl ether  
 3,3'-bis(m-phenoxyphenylmercapto)diphenyl ether  
 and  
 3-(m-phenoxyphenylmercapto)-3'-(m-phenoxy-  
 phenoxy)diphenyl sulfide.

In addition to the foregoing compounds, the phenyl and phenylene groups of such compounds can contain substituents, such as alkyl of one to four carbon atoms, alkoxy of one to four carbon atoms and halogen such as chlorine, bromine and fluorine. Examples of such compounds are as follows:

15 4,4'-bis(m-tolylmercapto)diphenyl ether  
 3,3'-bis(m-tolylmercapto)diphenyl ether  
 2,4'-bis(m-tolylmercapto)diphenyl ether  
 3,4'-bis(m-tolylmercapto)diphenyl ether  
 3,3'-bis(p-tolylmercapto)diphenyl ether  
 3,3'-bis(xylylmercapto)diphenyl ether  
 4,4'-bis(xylylmercapto)diphenyl ether  
 3,4'-bis(xylylmercapto)diphenyl ether  
 3,4'-bis(m-isopropylphenylmercapto)diphenyl ether  
 3,3'-bis(m-isopropylphenylmercapto)diphenyl ether  
 2,4'-bis(m-isopropylphenylmercapto)diphenyl ether  
 3,4'-bis(p-tert-butylphenylmercapto)diphenyl ether  
 4,4'-bis(p-tert-butylphenylmercapto)diphenyl ether  
 3,3'-bis(p-tert-butylphenylmercapto)diphenyl ether  
 3,3'-bis(2,4-di-tert-butylphenylmercapto)diphenyl  
 ether  
 3,3'-bis(3-chlorophenylmercapto)diphenyl ether  
 4,4'-bis(3-chlorophenylmercapto)diphenyl ether  
 3,3'-bis(m-trifluoromethylphenylmercapto)diphenyl  
 ether  
 4,4'-bis(m-trifluoromethylphenylmercapto)diphenyl  
 ether  
 3,4'-bis(m-trifluoromethylphenylmercapto)diphenyl  
 ether  
 40 2,3'-bis(m-trifluoromethylphenylmercapto)diphenyl  
 ether  
 3,3'-bis(p-trifluoromethylphenylmercapto)diphenyl  
 ether  
 3,3'-bis(o-trifluoromethylphenylmercapto)diphenyl  
 ether  
 3,3'-bis(m-methoxyphenylmercapto)diphenyl ether  
 3,4'-bis(m-isopropoxyphenylmercapto)diphenyl  
 ether  
 3,4'-bis(m-perfluorobutylphenylmercapto)diphenyl  
 ether  
 2-(m-tolylxy)-2'-phenylmercaptodiphenyl sulfide  
 2-(p-tolylxy)-3'-phenylmercaptodiphenyl sulfide  
 2-(o-tolylxy)-4'-phenylmercaptodiphenyl sulfide  
 3-(m-tolylxy)-3'-phenylmercaptodiphenyl sulfide  
 3-(m-tolylxy)-4'-phenylmercaptodiphenyl sulfide  
 4-(m-tolylxy)-4'-phenylmercaptodiphenyl sulfide  
 3-xylyloxy-4'-phenylmercaptodiphenyl sulfide  
 3-xylyloxy-3'-phenylmercaptodiphenyl sulfide  
 3-phenoxy-3'-(m-tolylmercapto)diphenyl sulfide  
 3-phenoxy-4'-(m-tolylmercapto)diphenyl sulfide  
 2-phenoxy-3'-(p-tolylmercapto)diphenyl sulfide  
 3-phenoxy-4'-(m-isopropylphenylmercapto)diphe-  
 nyl sulfide  
 3-phenoxy-3'-(m-isopropylphenylmercapto)diphe-  
 nyl sulfide  
 3-m-toloxo-3'-(m-isopropylphenylmercapto)diphe-  
 nyl sulfide

4-(m-trifluoromethylphenoxy)-4'-phenylmercapto diphenyl sulfide  
 3-(m-trifluoromethylphenoxy)-4'-phenylmercapto diphenyl sulfide  
 2-(m-trifluoromethylphenoxy)-3'-phenylmercapto diphenyl sulfide  
 3-(m-trifluoromethylphenoxy)-3'-phenylmercapto diphenyl sulfide  
 3-(p-chlorophenoxy)-3'-phenylmercapto diphenyl sulfide  
 3-(m-bromophenoxy)-4'-phenylmercapto diphenyl sulfide  
 bis[m-(m-chlorophenoxy)phenyl]sulfide  
 m-bis[3-(p-methylphenylmercapto)phenoxy] benzene  
 m-bis[3-(m-trifluoromethylphenoxy)phenylmercapto]benzene  
 m-bis[3-(m-bromophenoxy)phenylmercapto]benzene  
 3,3'-bis[m-(p-methylphenylmercapto)phenoxy] diphenyl sulfide  
 3,4'-bis[m-(p-methylphenylmercapto)phenoxy] diphenyl sulfide  
 3-(p-xenoxy)-3'-phenylmercapto diphenyl sulfide, and the like and mixtures thereof. It is also contemplated within the scope of this invention to employ mixtures of polyphenyl ether-thioethers as base stocks.

The compositions of this invention are useful as lubricants under extreme conditions. The compositions are especially useful for lubrication of steel on steel, silvered bronze, cast iron and the like.

#### EXAMPLE 1

A polyphenyl thioether - polyphenyl ether-thioether lubricant composition is prepared by combining phenyl phosphinic acid (0.075 gram) with 100 grams of a thioether of the following composition:

|                                                |                    |
|------------------------------------------------|--------------------|
| meta-bis(phenylmercapto)benzene                | (50% by weight)    |
| bis(phenoxyphenyl)sulfide                      | (12.5% by weight)  |
| (phenoxyphenyl) (phenylmercapto phenyl)sulfide | (23.5% by weight)  |
| bis(phenylmercaptophenyl)sulfide               | (12.65% by weight) |
| 3 ring and 5 ring thioethers                   | (1.35% by weight)  |

and containing 10 parts per million of a dimethyl silicone antifoam agent (Dow-Corning - 200, 350 cs. fluid).

The mixture was tested for lubricity on a high temperature wear machine. This machine comprises a steel shaft rotating on a silvered bronze disc so that there is line contact between the shaft and the disc. This test simulates the cage wear of silver plated bronze bearing cages. A lever movable about an axis permits the test disc to be loaded against the test shaft. The heated steel shaft (640° F.) is rotated against the disc at 30,180 rpm's at a load of 2.25 dekanewtons while the contacting surfaces are lubricated with the test oil at a flow rate of 1 ml. per minute. In the test the shaft requires 1 minute rotation to reach speed (30,180 rpm) and is maintained at this speed for 5 minutes and is then allowed to coast to a stop (1 minute). The wear scar is then measured. A test failure is indicated by seizure of the shaft and disc or an excessive wear scar.

When the mixture of Example 1 was tested at 640° F., the shaft did not seize and the scar wear was not excessive.

When the base fluid without the phenyl phosphinic acid was tested at 640° F. it failed the test.

The lubricating ability of the fluid from Example 1 was also shown with a slow speed four ball machine. A slow speed four ball machine measures the boundary lubricity action of additives. This test is a variation of the well known Shell Four Ball Test in which a ball is rotated against three stationary balls. Wear scars and/or seizure loads measure additive lubricity. In the slow speed instrument the three stationary balls are replaced with circular discs. Standard operating conditions are:

3 Kg. Load

1 r.p.m.

Room temperature to 700° F.

The speed of rotation is very low, namely one r.p.m. This equals 0.88 inches/minute. This is done for two reasons. It insures boundary conditions, i.e., metal to metal contact. It also eliminates metal skin temperature flashes which can occur at high speeds. Thus the bulk oil temperature is equivalent to the metal surface temperature. Under these conditions wear is negligible and friction is used to follow lubrication. After covering the ball and disc with the test oil, the initial friction is recorded. The test sample is then heated to 700° F. with continuous recording of the friction. This gives a boundary friction-temperature profile for the experimental fluid over this temperature range.

The mixture of Example 1 was tested by this procedure on 316 stainless steel. The coefficient of friction observed was always between 0.30 and 0.66 from room temperature to 700° F.

When the base fluid without the phenyl phosphinic acid was tested under the same conditions the coefficient of friction showed a steep increase as the temperature was increased and exceeded 2.0.

The lubricating ability of the composition of Example 1 was also shown by a high speed Falex Test employing an M-10 steel pin and Meehanite cast iron blocks. The composition of Example 1 had a failure loss of 180 psi whereas the composition without the phenyl phosphinic acid additive failed at 25 to 50 psi.

A fluid composed of the base oil from Example 1 but containing 0.1 percent by weight of phenyl phosphinic acid as the lubricity additive was run in slow speed four ball test using M-50 steel for the ball and discs. This fluid had a lower boundary friction than the unblended oil from 200° F. to 500° F. and from 600° to 700° F. At no temperature from room temperature to 700° F. did the friction of the blend significantly exceed that of the base stock.

It will be appreciated that the composition of the invention, in addition to the polyphenyl thioether base fluid and the organic phosphinic acid additive, may also contain other additives, such as oxidation inhibitors, rust and corrosion inhibitors, antifoaming agents, detergents, viscosity index improvers such as polymeric materials for example, polyacrylate alkyl esters, polymethacrylate alkyl esters, polyoxyalkylene compounds, polyurethanes and the like. Such additives are usually employed in amounts as low as 10 parts per million for antifoaming agent to as much as 15 parts by weight of the total compositions for viscosity index improvers.

While this invention has been described with respect to various specific examples and embodiments, it is understood that the invention is not limited thereto and that it can be variously practiced within the scope of the following claims.

The embodiments of this invention in which an exclusive property or privilege is claimed are defined as follows:

1. A lubricant composition consisting essentially of a major amount of a polyphenyl thioether having the formula



wherein R is a phenyl group or a substituted phenyl group, R' is a phenylene group or substituted phenylene group, in which the substituents on said phenyl and phenylene groups are halogen, alkyl or alkoxy containing from one to four carbon atoms, n is an integer of from one to six, Y is sulfur or oxygen provided that at least one of the groups represented by Y is sulfur, and mixtures of such thioethers and from about 0.05 to about 2.0 percent by weight of an organic phosphinic acid of the formula



wherein R'' is an aryl group containing from six to sixteen carbon atoms, a halogen substituted aryl group containing from six to sixteen carbon atoms, an alkyl substituted aryl group containing from six to 16 carbon atoms or an alkyl group containing one to 12 carbon atoms.

2. A composition of claim 1 wherein said organic phosphinic acid is present in amounts of from about 0.075 to about 0.2 percent by weight.

3. A composition of claim 1 wherein said organic phosphinic acid is phenyl phosphinic acid.

4. A composition of claim 2 wherein said organic phosphinic acid is phenyl phosphinic acid.

5. A composition of claim 1 where n is from one to three.

\* \* \* \* \*